

## UNITED STATES PATENT OFFICE.

MYRON PARK DAVIS, OF YONKERS, NEW YORK, ASSIGNOR TO OTIS ELEVATOR COMPANY, OF JERSEY CITY, NEW JERSEY, A CORPORATION OF NEW JERSEY.

## CUTTING OIL AND PROCESS OF PRODUCING SAME

No Drawing.

Application filed February 3, 1926 Serial No. 85,750.

The present invention relates to the production of compounded oils in general, and more particularly to the class of oils known as cutting oils. Important objects of this invention are to produce a superior quality of cutting oil and to provide an improved process for the production of such oil.

According to a specific example of the present invention, the compounded oil is produced by introducing flowers of sulphur into lard oil and thereafter combining the resultant product with a mineral or paraffin oil.

In carrying out the process, one may proceed as follows: 10 gallons of a fat oil such as lard oil are heated to a temperature in the neighborhood of from 450° F. to 475° F., the oil being thoroughly agitated during the heating operation to obtain uniform heating throughout. The application of heat is then discontinued and twenty pounds of finely divided flowers of sulphur are very carefully stirred into the fat oil. A foaming will shortly commence and this foaming is allowed to proceed for a few minutes after which a small amount of paraffin oil (for example 1 to 2 gallons of paraffin oil of a viscosity in the neighborhood of 100 seconds at 100° F. Saybolt standard) is slowly added while stirring. This addition of the paraffin oil will cause the foaming or reaction to subside. The stirring of the oil is still continued and shortly a second foaming will start, which is allowed to progress until it subsides of its own accord and then from 3 to 5 gallons additional quantity of the paraffin oil above referred to is carefully and slowly added while continuing the stirring. After all action has subsided, the mixture is diluted with the paraffin oil in further quantity, as above, until a total desired volume of, for example, 50 gallons is obtained.

During the compounding, it is important that the oil should at all times be kept in a state of agitation.

After the last addition of paraffin oil has been completely incorporated, the oil is then ready for use or for storing in containers.

Compounded lubricating oil produced according to the present process contains a high proportion of sulphur and exhibits superior properties or qualities as a cutting oil.

It will be understood that the above example which has been specifically given is intended only as an illustration of the principles involved in the invention, and that modifications may be adopted within the principle illustrated to conform with special requirements, without departing from the spirit of the invention.

What is claimed is:

1. The process of compounding cutting oil, which comprises heating a lard oil to a temperature in the neighborhood of from 450° F. to 475° F., while thoroughly agitating the same, discontinuing the heating and introducing finely divided flowers of sulphur in the proportion of approximately 20 pounds of sulphur to 10 gallons of lard oil with thorough agitation, allowing the resulting action to continue for a few minutes and thereafter adding paraffin oil of a viscosity in the neighborhood of 100 seconds at 100° F. Saybolt standard until 4 to 7 gallons of paraffin oil are added to each 10 gallons of lard oil, continuing to stir the mixture while the reaction proceeds, and after all action has subsided diluting the material with a further quantity of paraffin oil to a total volume of approximately 50 gallons for each 10 gallons of lard oil.

2. In the process of compounding cutting oil, the steps which comprise heating and agitating lard oil at a temperature in the neighborhood of from 450° F. to 475° F., discontinuing the application of heat, and introducing finely divided flowers of sulphur into the hot lard oil in the proportion of approximately 20 pounds of sulphur to 10 gallons of lard oil, and thereafter adding paraffin oil in the proportion of from 1 to 2 gallons of paraffin oil to 10 gallons of lard oil.

In testimony whereof, I have signed my name to this specification.

MYRON PARK DAVIS.